

## UNITED STATES PATENT OFFICE

2,355,242

## ASPHALT COMPOSITION CAPABLE OF COLD APPLICATION

Joseph C. Roediger, Brooklyn, N. Y., assignor to Standard Oil Development Company, a corporation of Delaware

No Drawing. Application December 19, 1940,  
Serial No. 370,785

2 Claims. (Cl. 106—280)

This invention relates to improvements in the preparation of asphalt compositions and particularly to asphaltic compositions that may be prepared and applied cold and which are capable of setting on standing without subsequent application of heat or pressure.

It has always been desirable to have an asphaltic composition that may be used while cold as a coating or bonding agent composed of mineral aggregate, fibrous material and other solids. The high temperatures required for the application of relatively high consistency asphalts (above 100° F. softening point) becomes hazardous in certain locations where explosive vapors exist. Although these asphalts may be applied at ordinary temperatures by prior combination with a volatile solvent, this is undesirable on many installations, especially those involving porous surfaces, because of the absorption and retention of the solvent for long periods after application.

It is the object of this invention to provide an asphaltic composition that may be applied to any surface and which on standing, sets. Another object of this invention is to provide an asphaltic composition that may be applied with a trowel or mixed with granular materials and on subsequent standing, form a coating of the desired consistency. Another object of this invention is to provide means by which setting characteristics of the asphaltic composition can be suitably retarded to permit its storage without setting for reasonable periods of time after mixing the various ingredients.

According to this invention in cases where it is desired to apply an asphalt of relatively high softening point and application cannot be made with the asphalt in a cutback or molten state, the following procedure can be used: a finely powdered, high softening point asphalt is mixed,

etc. On subsequent standing, the hard asphalt and the flux knit together to form an asphalt of the desired consistency regulated by the type, consistency and relative percentages of the two materials blended.

For example, 51 parts by weight of a reduced gas oil tar having a viscosity of 175 Furol at 122° F. were mixed with 10 parts of finely divided asbestos fiber and 39 parts of a 350° F. softening point tar asphalt prepared by vacuum reduction of a mixture of reduced and gas oil tars. This mixture could be readily trowelled for a period of several hours after incorporation of all the ingredients and when applied to a vertical metal surface adhered well and did not flow. This mixture gradually hardened so that after one week a substantially hard film developed. On continued exposure, the complete fluxing of the two asphaltic materials should produce an asphalt of approximately 125° F. softening point and 51 penetration at 77° F.

With mineral aggregates similar results can be obtained. Ninety-four parts by weight of standard Ottawa sand were mixed with a low consistency flux oil and after uniform coating the proper amount of finely, pulverized hard asphalt was added and mixed. The total of the hard asphalt and flux oil employed was equivalent to six parts by weight of the mixture, the relative proportions of both asphalts being regulated so that asphalt of 51/60 penetration at 77° F. would result on complete fluxing. Briquettes one-inch high and two-inches in diameter were prepared and their strength determined after various periods of storage at room temperature using the Hubbard-Field stability apparatus. The strength data given below show that the rate of setting of the mixtures can be regulated by changes in the source and consistency of powdered hard asphalt and the flux oil.

|   | Hard asphalt                                      | Fluxing oil      |                 | Hubbard-Field stability |             |              |
|---|---------------------------------------------------|------------------|-----------------|-------------------------|-------------|--------------|
|   |                                                   | Type             | Furol V/122° F. | Immediately             | After 1 day | After 6 days |
| 1 | 185 S. P. reduced gas oil tar                     | Red. gas oil tar | 175             | 350                     | 725         | 800          |
| 2 | do                                                | do               | 916             | 50                      | 200         | 300          |
| 3 | 250 S. P. reduced gas oil-reduced crude tar mixt. | do               | 175             | 175                     | 325         | 325          |
| 4 | do                                                | do               | 916             | 100                     | 220         | 260          |
| 5 | 235/250 S. P. oxidized Venez. asp.                | do               | 916             | 125                     | 180         | 450          |

directly prior to use, with an asphaltic oil of suitable viscosity. The mixture can be applied by trowel or mixed with granular material such as sand, mineral aggregate, asbestos, ground cork,

This procedure also can be employed when cellulosic materials such as cork are to be bonded with asphaltic material since the use of high temperatures normally necessary to incorporate high

consistency asphalt may have an injurious effect on cork.

When the asphaltic material is to be stored for appreciable lengths of time before use, the setting characteristics can be further regulated by:

1. Mixing mineral aggregate with a small amount of water containing an emulsifier such as alkali soaps, sulfonate soaps, etc., then adding a suitable quantity of low consistency flux oil and continuing the mixing so that an emulsion of the flux oil in the water solution of emulsifier is formed on the mineral aggregate. Following this, a high softening point, powdered asphalt is added and incorporated into the mixture. Due to the dispersed condition of the flux oil, considerable time will ensue before the emulsion breaks (either by subsequent drying when spread or by chemical action), so that the flux oil can contact the hard asphalt. A mixture so prepared should have slow setting characteristics permitting stock-piling for longer periods of time than now is possible with cutback asphalt, or ordinary flux oil-hard asphalt mixtures.

2. Preparing a dispersion of the low consistency flux oil in water with suitable emulsifiers first, and then applying this emulsion to the aggregate before final addition of powdered hard asphalt.

The dispersion of the flux oil in the water may be accomplished by the use of emulsifiers such as the sulfonate soaps, or other materials with which emulsions of relatively low pH may be prepared. This should be an advantage with certain aggregates where the presence of high pH materials such as sodium oleate, etc., is detrimental to the adhesivity of final asphalt film.

Varying the ratio of water to flux oil used in the mixture may be a means of controlling the setting characteristics of the final mixture, i. e., the higher the ratio of water, the slower should be the setting rate of the final mixture, within, of course, the practical limits of usage.

The proportions of hard asphalt and flux oil may be varied to result in a final asphalt of the desired consistency after the two ingredients have completely blended.

I claim:

1. An asphaltic composition which is capable of setting and hardening on standing without the application of heat or pressure which comprises about 51 parts by weight of a reduced oil tar having a Furol viscosity of 175 seconds at 122° F., about 10 parts of finely divided asbestos fiber and about 39 parts of a powdered petroleum asphalt of 350° F. softening point tar asphalt prepared by vacuum reduction of a mixture of reduced crude and gas oil tars.

2. An asphaltic composition of about 125° F. softening point and about 51 penetration at 77° F. which is capable of setting and hardening on standing without the application of heat or pressure, which comprises about 51 parts by weight of a reduced oil tar having a Furol viscosity of 175 seconds at 122° F. and about 39 parts of a powdered petroleum asphalt of 350° F. softening point tar asphalt prepared by vacuum reduction of a mixture of reduced crude and gas oil tars.

JOSEPH C. ROEDIGER.